

April 28, 1970

E. J. MELLEN, JR., ETAL

3,508,602

PERMEABLE SHELL MOLDS

Original Filed Dec. 2, 1965

2 Sheets-Sheet 1



Fig. 1



Fig. 2



Fig. 3



Fig. 4



INVENTORS  
EDWARD J. MELLEN JR.  
EDMOND M. BAKER  
JOHN M. WEBB  
Mc Coy, Greene & Howell  
ATTORNEYS

April 28, 1970

E. J. MELLEN, JR., ET AL

3,508,602

PERMEABLE SHELL MOLDS

Original Filed Dec. 2, 1965

2 Sheets-Sheet 2



Fig. 6



Fig. 7



Fig. 8



Fig. 9



Fig. 10

INVENTORS  
EDWARD J. MELLEN JR.  
EDMOND M. BAKER  
JOHN M. WEBB  
McCoy, Greene & Howell  
ATTORNEYS

## 1

3,508,602

## PERMEABLE SHELL MOLDS

Edward J. Mellen, Jr., 2123 Lee Blvd., East Cleveland, Ohio 44112, and Edmond M. Baker, Alliance, and John M. Webb, Chagrin Falls, Ohio; said Baker and said Webb assignors to said Mellen  
Original application Dec. 2, 1965, Ser. No. 511,129, now Patent No. 3,452,804, dated July 1, 1969. Divided and this application Dec. 4, 1968, Ser. No. 781,069  
Int. Cl. B22c 9/04

U.S. CL. 164—361

16 Claims

## ABSTRACT OF THE DISCLOSURE

A shell mold, ladle, crucible or the like made by dipping a destructible form or pattern in a ceramic slurry, randomly applying short threads or filaments to the resulting refractory layer so that they project outwardly from said layer in all directions, wrapping a destructible rope or cord around the ceramic-coated form or pattern to provide a closely spaced network, forming a series of ceramic coats which cover the network and the threads to form a ceramic article of substantial thickness by repeatedly dipping the pattern in the ceramic slurry, and firing the resulting ceramic article to burn out the rope.

This application is a division of our copending application Ser. No. 511,129, filed Dec. 2, 1965, now Patent No. 3,452,804, issued July 1, 1969.

The present invention relates to refractory molds having improved strength and permeability produced by repeatedly dipping a removable or destructible pattern in a ceramic slurry and more particularly to refractory investment molds made by wrapping the coated pattern with a destructible rope or cord and/or covering the coated pattern with short threads or filaments before all of the refractory material is applied.

Heretofore investment shell molds have been produced by repeatedly dipping a pattern of frozen-mercury, wax or other destructible material in a ceramic slurry and drying each layer to produce 4 to 10 or more layers with a total shell thickness of  $\frac{1}{4}$  to  $\frac{1}{2}$  inch or more. If desired, each slurry layer was dusted with dry refractory particles before drying of that layer. After the mold was built up to the desired thickness, the pattern was removed in a suitable manner, as by melting or dissolving it, the mold was fired, and thereafter the mold was preheated and filled with molten metal to effect casting of the desired metal article.

In order to obtain satisfactory results by the shell molding process it was necessary to provide the mold with adequate strength, porosity and resistance to thermal shock and to provide the mold cavity with dimensional accuracy and proper surface finish. The "lost-wax" shell molding process was not satisfactory for making some types of articles, especially those of very large size, because these problems were not solved.

The problem of producing large shell molds economically with adequate green strength, porosity and resistance to cracking has been recognized for many years, but a simple and practical solution to this problem was not found prior to the present invention. It has now been discovered that excellent shell molds for very large castings can be made in a simple manner by employing destructible threads or fibers to reinforce the green mold, to improve the porosity of the mold, and to reduce the weight of the mold for a given wall thickness. The process of this invention improves both small and large shell molds and makes it possible to cast the metal at room tempera-

## 2

ture without preheating the shell mold, as was necessary prior to this invention, and without a backing for the shell mold.

When making shell molds by the process of this invention, the prime dip coats may be applied to the pattern in the usual manner, with or without dusting, to provide the shell mold with the desired internal surface characteristics. Thereafter, cords or threads of a suitable destructible material, such as stiff natural or synthetic fibers are secured in outwardly projecting positions to the coated pattern, and additional layers of refractory material are applied in a conventional manner to build up the desired thickness of the shell wall. The destructible threads may be applied by a sprinkling or "flocking" operation after dipping the coated pattern in the ceramic slurry.

When making a large shell mold, it is preferable to apply a destructible fiber twine or other rope to the partially formed shell mold so that the ceramic slurry subsequently applied will penetrate the interstices thereof.

The rope is preferably wound around the pattern to provide a network of closely spaced portions or strands reinforcing the mold, and additional destructible material is preferably sprinkled on the mold in the form of short threads or fibers to provide additional green strength and to improve further the porosity of the mold after firing. In this way it is possible to maintain dimensional accuracy and to avoid damage to the shell mold during the dipping, dusting, drying and pattern removal operations and to provide a durable mold which is strong enough for pouring of a very heavy casting, which can withstand high thermal shocks, and which, nevertheless, has very high permeability. Upon firing of the "green" shell mold, the rope or twine is burned leaving passages for flow of gas into or out of the mold. These passages are smaller than the external dimensions of the rope or twine because the ceramic material penetrates the interstices of the cord and, therefore, the passages do not weaken the mold but have a tendency to further strengthen it. The short destructible threads applied to the shell mold are also burned out to provide small passages for escape of gas from the mold during the metal casting operation.

The ceramic impregnated rope or twine and/or the destructible threads or fibers burn out much slower than a wax pattern and retain their strength long enough to resist cracking of the mold during the wax removal process.

If desired, the destructible rope or twine used in making the shell molds of this invention may be coated with an organic material of high boiling point, such as tar or pitch, to produce a reducing atmosphere during casting of the metal in the shell molds.

An object of the invention is to provide a simple inexpensive refractory mold for making large-size precision metal castings which can be made without expensive equipment.

A further object of the invention is to improve the permeability of shell molds and to speed up removal of gas from a shell mold when pouring molten metal into the mold.

Another object of the invention is to improve the green strength of shell molds and to avoid cracking of the molds.

Another object is to provide voids, left from the rope which permit passing any type of gas such as a reducing gas, through the mold just before or during casting.

Another object of the invention is to provide a mold reinforcement which does not interfere with bonding of one ceramic layer to the next and which burns out at a slower rate than the wax pattern so as to reinforce the mold during wax removal.

Another object is to provide a mold which permits a method of dewaxing which is more economical than the conventional flash firing method.

Another object of the invention is to prevent mold distortion and provide large precision castings with close tolerances.

A still further object of the invention is to eliminate the need for preheating of shell molds prior to metal casting.

Another object of the invention is to provide high strength investment shell molds suitable for vacuum casting.

These and other objects, uses and advantages of the invention will become apparent from the following description and claims and from the drawings, in which:

FIGURE 1 is a perspective view showing a conventional wax pattern on a reduced scale;

FIGURE 2 is a perspective view showing a ceramic-coated wax pattern with a supporting rope attached thereto according to the process of this invention;

FIGURE 3 is a top plan view of the rope-reinforced pattern of FIGURE 2;

FIGURE 4 is a schematic top plan view similar to FIGURE 3 but showing the positions of reinforcing ropes forming a network on the top surface of the pattern;

FIGURE 5 is a schematic bottom view of the rope-reinforced pattern of FIGURE 4 showing the rope network on the bottom surface of the pattern;

FIGURE 6 is a fragmentary vertical sectional view of the rope-reinforced pattern of FIGURES 2 and 3;

FIGURE 7 is an enlarged fragmentary sectional view of the shell mold made by the process of FIGURES 2 to 6 prior to firing of the mold;

FIGURE 8 is a perspective view of the completed shell mold made by the above process;

FIGURE 9 is a perspective view of another form of conventional wax pattern on a reduced scale; and

FIGURE 10 is perspective view of the finished shell mold formed on the wax pattern of FIGURE 9 by the process of this invention.

Referring more particularly to the drawings, FIGURE 1 shows a conventional wax pattern A in the form of a large turbine blade wheel having a flat disc-shaped portion 1, a tapered hub portion 2, and a series of regularly spaced curved blade slots 3 of generally uniform width. A conventional supporting hook 4 is embedded in the pattern.

In performing the process of this invention, one or two prime dip coats are applied to the wax pattern, and the coated pattern is then reinforced by a rope network, which may be applied by extending portions of the rope through the slots 3. FIGURES 2 through 6 show one way in which the reinforcing twine or other rope may be applied, it being understood that many other arrangements of rope are also suitable.

FIGURE 2 shows how supporting ropes may be attached to the base of the hook member 4. Thus, the rope may be extended radially outwardly from the base of the hook over the portion 1 to the outer margin of the pattern, under the pattern to the adjacent slot 3, and through that slot to another slot, thereby forming the three rope portions 5, 6 and 7 (see FIGURE 6). The rope portion 8 then returns to the hook 4 and remaining portions of the rope are used in a similar manner to form the radial portions 9, 11, 12 and 14 and the horizontal intermediate portions 10 and 13 as indicated in FIGURES 2 and 3. Although the intermediate portions 7, 10 and 13 are shown herein as effecting the attachment of the pattern, it will be apparent that the rope can be tied around the pattern in various other ways.

As shown diagrammatically in FIGURES 4 and 5, a rope network 29 is formed on the flat bottom surface of the pattern and a rope network 30 is formed on the flat upper surface of the disc portion 1. While the rope should be sufficiently taut, it should not be so tight that it could

distort the pattern or crack the mold. The various ropes of the network are shown schematically by solid lines, the arrows indicating the direction in which the rope may be extended when it is applied. Obviously almost all of the two rope networks 29 and 30 may be formed from one long piece of twine or other rope, but more than one piece of rope is usually employed. Also, the networks may be preformed before being attached to the pattern if this is desired. Thus good results can be obtained using fishnets or the like with a spacing of  $\frac{1}{4}$  inch to 1.5 inches between cords.

When applying the network as shown in FIGURE 4 and 5, the twine or other rope is extended through the outer ends of the slots 3 identified by the numerals 21 through 28 and around portions of the pattern to provide short marginal rope portions 36 and 38 adjacent the upper and lower surfaces, respectively, of the disc portion 1 and longer marginal rope portions 37 and 39 adjacent the lower and upper surfaces, respectively, of said disc portion. The rope portions 36 through 39 thus provide points of attachment at the slot ends 21 through 28.

It can readily be seen how a rope network may be formed by using such attaching points. Thus, as indicated in FIGURE 5, the network 29 is formed by extending one piece of rope from the slot end 23 to the end 27 to form the rope section a, extending it to end 19 to form section b, then extending it from 19 to 24 to form section c, and continuing to extend the rope past points 22, 20, 26, 17, 30, 28, 18 and 25 to form the rope sections d through k. Additional pieces of rope may be arranged in a generally similar manner to complete the network 29 as shown in FIGURE 5. The network 30 may be formed in a similar manner on the upper surface of the disc portion 1 using the attaching points 21 through 28 at said upper surface as shown in FIGURE 4. Portions of the rope may extend around the hub 2 to reinforce the pattern in this area, but this is not essential.

The rope sections of each network are preferably closely spaced, best results usually being obtained when the ropes are spaced apart about one to two inches. When practicing the present invention, it is desirable to divide the surface of the pattern into squares with a width of about  $1\frac{1}{2}$  inches, where it is convenient to do so, but, with some patterns, various other arrangements are preferred.

After the rope networks are applied to the upper and lower surfaces of the destructible pattern, the additional layers of ceramic material necessary to give the shell mold the desired thickness are applied in the conventional manner as described in more detail hereinafter, preferably after sprinkling short destructible threads or fibers over the pattern. The finished shell mold is shown in FIGURES 7 and 8, prior to removal of the pattern and firing of the mold.

The process of this invention is particularly well suited for use with wax patterns but may be used with patterns made of synthetic resins, mercury, mercury alloys or other destructible materials. Any conventional ceramic materials and binders may be employed to make the shell molds of this invention. Suitable ceramic slurries are disclosed, for example, in the following U.S. Patents Nos. 2,806,269; 2,818,619; 2,911,310; 2,913,729; 2,961,751; 2,932,864 and 3,160,931. Good results can be obtained using ceramic slurries of the general type disclosed in the co-pending allowed application of E. J. Mellen et al., Ser. No. 276,753, filed Apr. 30, 1963, now Patent No. 3,222,435.

In order to obtain a good surface finish on the casting, it is desirable to use refractory granules in the prime dip and the first dusting operation which are much finer than those used in the later-applied concrete dip slurries. Thus, all of the refractory particles used in the prime dip slurry may, for example be small enough to pass through a 200-mesh sieve. However, the refractory material of the con-

crete dip slurry may, for example, be such that no more than 50 percent by weight can pass through a 200-mesh sieve and the remainder will pass through a 50-mesh sieve.

The refractory material used in each slurry may be any conventional ceramic material used for making shell molds including zirconite, fused silica, aluminum silicate, zirconium silicate, alumina, etc. and any conventional binder may be used such as ethyl silicate, colloidal alumina, sodium silicate, colloidal zirconium, colloidal silica, etc. Both a low-temperature binder and a high-temperature binder may be employed as is well understood in the art.

The ceramic slurries may be applied by spraying or in any other suitable manner and may be dried in various ways with air or other gas. The preferred procedure is to dip the destructive pattern in the slurry and to evaporate the water or other slurry vehicle in air having a predetermined humidity and temperature. When using wax patterns it is desirable to effect dusting and drying using the process of U.S. Patent No. 2,932,864.

The term "drying" is used herein in the normal sense to describe the evaporation of most of the slurry vehicle and does not require removal of 100% of the liquid. The amount of drying should be sufficient to permit proper application of the next ceramic layer.

Although the ceramic slurry used for forming shell molds on the wax patterns may be any of the conventional materials used for this purpose, it is necessary to provide a slurry of the proper consistency. If a slurry is too thick, this can cause building up the thickness of the layers on the mold too rapidly. If, for example, the slurry contains too much of an organic material, such as a synthetic resin, it may be unsatisfactory. For this reason such resins are preferably omitted and, if used, are used in very small amounts.

Conventional hydrolyzed solutions of ethyl silicate are excellent for use in practicing the present invention although various other binders are equally suitable. The ethyl silicate type of binder usually comprises about 30 to 60% by weight of ethyl silicate (about 30 to 40%  $\text{SiO}_2$ ), about 30 to 60% alcohol, about 0.5 to 0.5% concentrated hydrochloric acid, and about one to 10% of water. One part by weight of such binder is usually mixed with about 2.5 to 4.5 parts by weight of the dry refractory material. Various catalysts and/or accelerators may be employed with the ethyl silicate binder including magnesium oxide, aluminum oxide, aluminum hydroxide, ammonium carbonate, ammonium acetate, morpholine, etc. Each ceramic layer of the shell mold made by the process of this invention is preferably made by applying the slurry to the pattern, draining off the excess slurry, and applying a stucco coat before drying the layer in a suitable dusting apparatus. The dusting steps speed up the formation of the shell mold, but it will be understood that dusting is not essential in the practice of this invention. It will also be apparent that any suitable method may be employed to evaporate the slurry vehicle from the individual ceramic layers and that each layer does not have to be dried 100% before applying the next layer. It is preferred to dry the mold rapidly using equipment of the type disclosed in said U.S. Patent No. 2,932,864, Patent No. 3,191,250 or Patent No. 3,307,232 but the patterns may be dried slowly, particularly when they are extremely large.

In practicing the process of the present invention, a typical procedure is to apply one or two prime dip layers to the removable or destructive pattern before applying the reinforcing rope or the destructive threads, each layer being formed by dipping the destructive pattern in the prime dip slurry, draining the excess slurry, dusting with fine ceramic particles and drying the individual layer in air or other gas. After the second layer is dried, the pattern may be dipped in the concrete slurry or the prime dip slurry, just prior to the application of the destructive threads. If reinforcing ropes are to be employed, then these are preferably applied before the flocking operation

is performed. After the pattern has been covered with the destructive fibers, conventional air drying may be employed with or without dusting. Thereafter several ceramic layers are preferably built up over the destructive threads or the reinforcing rope or both in conventional manner to provide the shell mold with the desired thickness. The total number of layers may vary from 4 to 10 or more. Usually each of the concrete slurry layers is formed by dipping the pattern in the concrete slurry, draining the excess slurry, dusting with coarse refractory particles, and evaporating the slurry vehicle with air. Dusting is preferably omitted after the last dip coat. In some cases post-fired dip coats may be used.

In practicing the present invention, it is preferable to apply the rope and/or the destructive threads or fibers after only one or two ceramic layers have been formed on the destructive pattern so that most of the layers of ceramic material are built up over the rope and/or the destructive fibers; however, it will be understood that more than one flocking operation can be employed and that the rope can be applied at different times during the building of the shell mold.

The twine or other rope and the short threads or filaments used in making the permeable shell molds of this invention may be formed of various destructive materials, such as natural and synthetic fibers or various metals. The fibrous material used may be cotton, wool, hair, silk, ramie, flax, hemp, jute, sisal, abaca, catgut, seaweed, cattail, milkweed, straw, grass, redwood bark, or other fibers of vegetable, mineral or animal origin. The fibrous material may be a protein fiber, such as one made from casein, soybeans, peanuts or corn, a cellulosic fiber such as viscose rayon or various other synthetic fibers. The short threads or filaments may also be made from quartz glass, fused silica or other ceramic, polystyrene, polyethylene, polyvinyl alcohol, cellulose acetate, cellulose butyrate, ethyl cellulose, acetate butyrate, polyamides such as nylon, vinyl resins, polyester resins, polyacrylic resins, natural rubber, synthetic rubbers, acetate rayon, polycaprolactam, or the like. The threads or filaments used in making the shell molds of this invention may be microbore quartz glass tubes or ceramic tubes of small diameter (e.g., a diameter of 0.04 to 0.1 inch) and need not be destructive. Such threads or filaments may be hollow or solid and may be only partially destructive. They may be common textile fibers or metal filaments which are chemically treated or coated with wax, ceramic or any other suitable material, such as a synthetic resin.

The metal used to form the rope or twine or the threads or filaments may be aluminum, brass, steel, iron, etc. It may, for example, be black iron or metal with a low coefficient of expansion, such as a non-expanding stainless steel. Good results can be obtained using wires or filaments made of a metal treated to form an oxide film on the surface. The rope or twine is preferably a hemp rope, nylon rope, binder's twine or the like and usually has a diameter of about 0.08 to 0.2 inch. If desired, the rope may be treated with asphalt, coal tar pitch or other suitable organic material to produce a reducing atmosphere in the mold when casting the metal. The amount of such material, of course, should not be excessive.

If the destructive material used to form the threads or fibers used in reinforcing the molds of this invention is not sufficiently stiff, it is possible for the threads to become matted or flattened on the surface of the coated pattern. This would cause weakening of the mold by interfering with the adhesion of subsequent ceramic layers and would not produce a satisfactory mold. Therefore, when using a material which is not stiff, the individual threads, fibers or filaments should be treated to obtain adequate stiffness as by coating with a synthetic resin or other suitable material. Of course such treatment is unnecessary when using stiff fibers, such as those made of hemp, jute, sisal, bassine, Tamico, redwood bark, straw or the like.

In practicing the process of this invention, fibers or filaments are used with a length of  $\frac{1}{4}$  to 1 inch or so having sufficient stiffness so as to remain in an outwardly projecting position when subsequent layers of ceramic material are applied, whereby the individual threads project through several layers of the ceramic material and help to prevent separation of the layers. Although minor amounts of fibers with a length somewhat less than  $\frac{1}{4}$  inch can be used in the practice of this invention, it is preferable to eliminate extremely short fibers because of their tendency to lay flat on the surface and interfere with adhesion of the next ceramic layer. Best results are usually obtained with fibers or filaments with a length of 0.4 inch to 1 inch.

To facilitate an understanding of the present invention, an example of the process of this invention is given below. A liquid carrier of prehydrolyzed ethyl silicate is prepared by mixing 5300 milliliters of ethyl silicate 40 (about 40%  $\text{SiO}_2$ ) with 4200 milliliters of ethyl alcohol and 500 milliliters of 1% hydrochloric acid. One part by weight of the resulting liquid carrier is then thoroughly mixed with 3 parts by weight of a conventional dry mix consisting of 65% by weight of zircon flour and 35% by weight of fused silica flour. Said flours are of a size to pass through a 325-mesh screen (standard Tyler sieve). The resulting ceramic slurry is employed as a prime dip slurry as indicated below.

In order to provide a concrete dip slurry containing a coarser refractory, the prehydrolyzed ethyl silicate prepared as indicated above is mixed with a coarse fused silica flour which will pass through a 120-mesh sieve. About one part by weight of the prehydrolyzed ethyl silicate solution is mixed with around 3 parts of the coarse silica flour and preferably with an amount which will provide a viscosity of 14 to 16 seconds using a standard #4 Zahn cup.

In forming the shell mold of this invention, the wax pattern A of FIGURE 1 is immersed in a dip tank containing the prime dip slurry described above, the solids preferably being kept in suspension (i.e., by rotating the tank continuously at a speed of about 30 r.p.m.). After dipping, the pattern is given a stucco coat and is air dried according to the method of said U.S. Patent No. 2,932,864. The dry refractory used for the first stucco coat is conventional and comprises 62.5 percent by weight of fused silica ( $-50 +100$  mesh) and 37.5 percent by weight of zircon sand ( $-80 +200$  mesh). After the first dipping, dusting and drying operation, the pattern is again dipped in the same prime dip slurry, dusted with the same dry refractory material and air dried in the same way and a  $\frac{1}{8}$  inch hemp twine (2-strand binder's twine) is mounted on the pattern over the resulting ceramic coating 15 as indicated in FIGURES 2 to 6.

After the hemp twine is applied, the rope-reinforced pattern is dipped, for example, in a rotating dip tank containing the concrete dip slurry described above and a stucco coat is applied by dusting using a suitable apparatus as disclosed in said Patent No. 2,932,864 but using a coarser refractory of a conventional type made by mixing 3 parts by weight of fused silica grains ( $-30 +50$  mesh) with 4 parts of calcined clay or grog (i.e., aluminum silicate). Of course, any coarse stucco material conventionally used for this purpose may be employed.

After the stucco is applied, air drying is effected according to the process of said Patent No. 2,932,864, and the pattern is again dipped in the same concrete slurry. Then the wet coated pattern is flocked by sprinkling ordinary bassine fibers with a length of about  $\frac{1}{2}$  inch over the entire outer surface of the coated pattern in such a manner that the fibers adhere to the wet ceramic outer layer and project outwardly therefrom. The application of the fibers may be effected using a conventional rotary dusting apparatus, such as that disclosed in said Patent No. 2,932,864, having buckets rotating with the drum which drop or sprinkle the fibers over the pattern. The

pattern may be rotated by hand as the fibers are applied, but this is not essential. After the fibers have been deposited on the wet surface, the pattern is again dipped in the concrete slurry, the excess slurry is drained off, and the wet pattern is dusted with the coarse ceramic particles and dried as before.

The dipping in the concrete slurry, the dusting with ceramic particles and the drying may be repeated to build up a total of 10 layers or so. Then the pattern is dipped in a ceramic slurry and dried without dusting to provide a final seal coat. The resulting shell mold is relatively thick in the vicinity of the individual rope sections and has a very irregular outer surface because of the projecting fibers 31 which project outwardly in all directions.

FIGURE 7 gives a general idea of the irregular shape of the shell mold prior to firing, it being understood that there are an infinite number of variations in the shape depending on the way in which the ropes and fibers are located.

As indicated in FIGURE 7, the reinforcing ropes of the network 30 are located near the upper surface 33 of the pattern and the ropes of the network 29 are located a short distance below the lower surface 34 of the pattern, the fibers 31 being closely spaced throughout the shell mold and providing a multiplicity of closely spaced projections 32 in the outer surface, said projections extending in all directions in a random fashion. Where the supporting rope sections 6 to 14 are employed, the radially extending sections will also be coated with refractory material to provide radial arms, such as the arms 6a, 11a, 12a and 14a.

The dried shell mold made as described above is then flash fired in a conventional manner at  $1850^{\circ}$  F. to effect removal of the wax and cooled to room temperature. This heating burns out the rope and the bassine fibers. However, the rope retains its strength longer than the wax and reinforces the mold so as to prevent cracking of the mold (i.e., due to expansion of the wax). The strength of the rope is not the only important factor, however, as the presence of the rope tends to provide an increase of the thickness and strength of the mold walls without a corresponding increase in the weight thereof.

The completed mold need not be preheated to effect casting of the metal as with conventional shell molds. Instead the metal may be poured into the mold while the mold is at room temperature. After pouring, the mold is cooled and the shell is broken away from the cast metal part.

Prior to this invention the conventional shell molds required higher pouring temperatures and preheating of the molds before metal casting. It was conventional to preheat the shell molds to about  $1800^{\circ}$  F. when pouring the metal at around  $3000^{\circ}$  F. The disadvantage of the preheating is that it requires an extra heating operation and sometimes tends to cause a reaction between the metal being cast and the material forming the mold. The process of this invention eliminates the need for the preheating operation and eliminates the metal mold reaction. Such preheating was necessary with conventional shell molds to facilitate removal of moisture and removal of air from the mold. This is not necessary with the mold of this invention because of the greater porosity of the mold caused by the ropes and fibers which burn out to leave voids in the wall of the mold and the reduced thickness of the shell mold between rope sections.

The highly porous molds of this invention are particularly good because they permit reduction in the metal pouring temperature. High pouring temperatures are undesirable for several reasons. For example, at high temperatures, some of the elements of the alloys, such as titanium or carbon, might be lost due to reaction with the container in which they were melted and other materials may be lost by vaporization. The hotter metal also tends to conform too closely to the rough surface of the mold cavity and to provide the casting with a correspondingly

rough surface. The porous molds of the present invention permit pouring of the metal and complete filling of the mold cavity when using lower pouring temperatures. The advantages of such lower temperatures are finer grain size, increased strength and better metal properties. There is produced a smoother surface on the casting, and there is less tendency of the metal to run into depressions or vent openings of the mold, such as those produced by the randomly disposed brush fibers.

The shell mold of this invention has other advantages. Because of the strong waffle-type wall structure it is unnecessary to provide a backing for the shell mold of this invention when casting the metal. While maximum reinforcement is obtained using ropes as disclosed, for example, in FIGURES 2 to 8, a very substantial reinforcement of the mold is obtained using fibers alone. FIGURES 9 and 10 illustrate this process when using a conventional wax pattern B in the form of a tree or cluster. The pattern B has a tapered central portion 51 of circular cross section having embedded therein a supporting hook 50. The pattern has a series of pattern members 52 of circular cross section regularly spaced around the circumference of the pattern B and held in position by a series of connecting portions 53 and a circular base portion 54. The pattern B is conventional and forms no part of this invention.

An example of the process of this invention using fibers only as the reinforcement is given below. The pattern B is dipped in the prime dip slurry, the excess slurry is drained off, a stucco coat is applied by dusting, using the fine ceramic material described above, and the coated pattern is air dried as described in the previous example. The dipping, draining, cutting, dusting and drying is repeated to form a second prime dip layer. Then the pattern B is dipped in the rotating dip tank containing the concrete dip slurry described above, the excess slurry is drained off and  $\frac{1}{2}$  inch bassine fibers 56 are sprinkled over the entire outer surface of the pattern by the method of the previous example so that the fibers project outwardly from the surface and do not interfere with adhesion of subsequent layers. The wet coated pattern is then air dried, and seven layers of concrete slurry are applied to complete the mold as shown in FIGURE 10. Each concrete layer is applied in the conventional manner by dipping in the concrete ceramic slurry, draining off the excess slurry, dusting with the coarse ceramic particles described above and air drying in the usual manner. The dusting operation is omitted when the last coat is applied.

The resulting shell mold is then flash fired at  $1850^{\circ}$  F. to effect wax removal. The mold is then cooled to room temperature, the molten metal is poured into the mold to form the desired metal casting. It is to be understood that the mold can be preheated to an elevated temperature before pouring, if so desired.

The fibers do not interfere with bonding of one ceramic layer to the next because they do not lay flat but project outwardly through the different layers. Thus, they extend through a series of layers and act like nails to hold the layers together and strengthen the mold instead of weakening it, as would be the case if resinous particles were mixed with or sprinkled on the ceramic material. The fibers greatly increase the strength of the mold in the green state and, because they burn out slower than the wax, they reinforce the mold to prevent cracking during wax removal.

Prior to this invention, steam degreasing or dewaxing was considered impractical because it cracked or damaged too many molds. The rope and fiber-reinforced shell molds of this invention resist such cracking and making it practical to disintegrate the pattern at atmospheric pressure using steam at a temperature in the neighborhood of  $212^{\circ}$  F. This permits use of more economical wax removal processes.

Heretofore, it was difficult to produce large castings having portions extending outwardly a substantial dis-

tance from a central support. In order to make shell molds for such castings on destructible patterns, it was considered necessary to provide a gating system wherein the gates were located at the margin of the article so as to function with a steel framework to provide support for the mold. This was expensive because of the cost of the additional wax and ceramic material, the special brackets or other framework, and the extra metal used during casting. The process of this invention eliminates the need for a wax pattern of such special construction and greatly reduces the cost of manufacture of large precision castings while making it possible to maintain close tolerances.

In practicing the present invention, use may be made of a twine or other rope which can absorb a substantial amount of the ceramic material. An advantage of having the ceramic material penetrate the rope is that the rate of burning of the rope is reduced. Thus, the rope is able to retain its strength for a longer period of time during removal of the wax or other destructible material to prevent cracking of the mold.

While the process of this invention is usually applied to the making of the more common types of investment shell molds it will be understood that it may be applied to crucibles used in induction furnaces for melting the metal, to ladles used to transport the molten metal from the furnace to the refractory molds and to other refractory articles. Thus where a crucible or ladle is made according to the process of U.S. Patent No. 2,932,864, its strength may be increased by the use of rope and/or fibers according to the process of the present invention.

The present invention may be practiced using any of the known binder systems and any of the known types of destructible patterns including frozen mercury patterns. The gelling of the ethyl silicate may, for example, be effected by use of ammonia vapors. Excellent shell molds may, for example, be made by the alternate dip method wherein each ceramic layer formed from the ethyl silicate slurry is followed by a layer formed from a colloidal silica slurry.

The short filaments used in making the molds of this invention are preferably solid, rather than hollow. When they are solid they are preferably formed of a destructible material rather than a refractory material.

Unless the context shows otherwise, all percentages given herein are by weight and "parts" means parts by weight.

It will be understood that the above description is by way of illustration rather than limitation and that, in accordance with the provisions of the patent laws, variations and modifications of the specific compositions, methods and products disclosed herein may be made without departing from the spirit of the invention.

Having described our invention, we claim:

1. A refractory shell mold for use in casting molten metal comprising a thick refractory body with a layer forming a smooth, continuous internal surface defining a mold cavity of a predetermined shape and an outer layer forming a rough outer surface, a network of closely spaced rope-shaped passages surrounding the mold cavity, and a multiplicity of closely spaced thread-like voids randomly distributed throughout said body and projecting outwardly to vent the mold cavity, said body having a series of refractory layers surrounding the mold cavity and covering said passages and said threadlike voids, said layers conforming generally to the contour of said passages and said voids, said outer layer projecting outwardly in the vicinity of said voids.

2. A refractory shell mold as defined in claim 1 wherein said threadlike voids have a length of about  $\frac{1}{4}$  inch to about 1 inch and are covered by 4 to 10 of said refractory layers.

3. A refractory shell mold as defined in claim 1 wherein said voids are formed by filaments which are at least partially destructible.

4. A refractory shell mold as defined in claim 1 wherein said voids are formed by metal filaments.

5. A refractory shell mold as defined in claim 1 wherein said voids are formed by ceramic filaments.

6. A refractory shell mold as defined in claim 1 wherein said voids are formed by silica glass tubes with a length of about  $\frac{1}{4}$  inch to about 1 inch.

7. A refractory shell mold as defined in claim 1 wherein said voids are formed by hollow ceramic tubes with a length of about  $\frac{1}{4}$  inch to about 1 inch.

8. A refractory shell mold as defined in claim 1 wherein said passages are formed by metal rope.

9. A refractory mold for use in casting molten metal comprising a thick refractory body with a layer forming a smooth continuous internal surface defining a mold cavity of a predetermined shape and an outer layer forming a rough outer surface, closely spaced rope-formed passages surrounding the mold cavity with a shape corresponding to that of the rope prior to firing, and a multiplicity of closely spaced threadlike voids with a length of about  $\frac{1}{4}$  inch to about 1 inch randomly distributed throughout said body and projecting outwardly through a series of ceramic layers to vent the mold cavity, said body having a series of refractory layer surrounding the mold cavity and covering said passages and said threadlike voids, said layers conforming generally to the contour provided by said passages and said voids and projecting outwardly in the vicinity of said voids.

10. A refractory mold as defined in claim 9 wherein said passages contain metal ropes which provide a reinforcing network above and below the mold cavity.

11. A refractory mold as defined in claim 9 wherein said passages have a shape corresponding to that of a fishnet having a spacing of about  $\frac{1}{4}$  inch to about  $1\frac{1}{2}$  inches between cords.

12. A mold as defined in claim 9 wherein said passages are formed by a rope made of black iron.

13. A mold as defined in claim 9 wherein said passages are formed by a stainless steel having a low coefficient of expansion.

14. A mold as defined in claim 9 wherein said passages are formed by ropes made of metal wires having an oxide film on the surface.

15. A multi-layer refractory shell mold for investment casting comprising a thick refractory body with a layer forming a smooth continuous internal surface defining a mold cavity of a predetermined shape and an outer layer forming a rough outer surface, a network of closely spaced passages formed throughout said body above and below said mold cavity by crossing rope sections and surrounded by ceramic material corresponding to that which penetrated the interstices of the rope, said body comprising a series of refractory layers surrounding the mold cavity, covering said network of passages, and conforming generally to the contour of said network.

16. A multi-layer shell mold as defined in claim 15 having 4 to 10 refractory layers and having external refractory cables formed by external rope strands and radially arranged to reinforce the mold, said rope strands being covered with a series of layers of refractory material.

#### References Cited

#### UNITED STATES PATENTS

|           |         |                     |           |
|-----------|---------|---------------------|-----------|
| 3,041,131 | 6/1962  | Juras et al. -----  | 164-43 X  |
| 3,066,365 | 12/1962 | Moore -----         | 164-43 X  |
| 3,166,808 | 1/1965  | Moore -----         | 164-41 X  |
| 3,367,393 | 2/1968  | Lenahan et al. ---- | 164-361 X |
| 3,374,825 | 3/1968  | Johnson -----       | 164-43 X  |

J. SPENCER OVERHOLSER, Primary Examiner

R. S. ANNEAR, Assistant Examiner